

Aug. 13, 1968

E. F. CHRISTIANSEN

3,396,447

METHOD OF DIFFUSION OF MOLYBDENUM INTO EXTRUDED  
FERROUS METAL SURFACES OF A PISTON

Filed Jan. 19, 1966



## 1

3,396,447

### METHOD OF DIFFUSION OF MOYBDENUM INTO EXTRUDED FERROUS METAL SURFACES OF A PISTON

Erik Frede Christiansen, Sonderborg, Denmark, assignor to Danfoss A/S, Patent Department, Nordborg, Denmark

Filed Jan. 19, 1966, Ser. No. 521,688  
Claims priority, application Germany, Jan. 30, 1965,  
D 46,396

7 Claims. (Cl. 29—156.5)

#### ABSTRACT OF THE DISCLOSURE

A method of diffusion of molybdenum into inter-atomic or inter-crystalline interstices of an extruded ferrous metal surface to decrease the coefficient of friction of the surface. Molybdenum or molybdenum-containing powder is kept in contact with the extruded ferrous surface and then the surface with the powder thereon is subjected to heat treatment. Because the extruded surface has been subjected to shear the surface is particularly susceptible to diffusion by molybdenum. The heat treatment may take place in an inert gas atmosphere or in the presence of a reducing gas.

This invention relates to a method for introducing molybdenum into a ferrous metal surface and to articles having such a surface into which molybdenum was introduced by the method of the invention. According to the invention, molybdenum is caused to diffuse into a surface of a ferrous metal article. Thus, the invention also relates to ferrous metal articles having molybdenum diffused into a surface thereof.

The expression "ferrous metal" is intended to denote iron and alloys of iron such as steels.

The primary object of introducing molybdenum into a ferrous metal surface according to the invention is to decrease the coefficient of friction of the surface. Thus, the invention is particularly useful where the ferrous metal surface is a surface of a machine part or element which slides along another machine part or element during the operation of the machine. Thus, for example, a surface which is treated according to the invention may be the peripheral surface of a piston which reciprocates in a cylinder, as for instance a piston for a compressor of a refrigerating unit.

It is known to provide running surfaces (i.e., surfaces which slidingly engage other surfaces) with molybdenum sulfide in order to decrease the coefficient of friction of the running surfaces. For example, molybdenum sulfide powder is rubbed into the surface or molybdenum tri-oxide is electrolytically deposited on the surface and is subsequently converted to molybdenum sulfide by exposure to a hydrogen sulfide atmosphere. However, the effective lives of these treatments are limited. Thus, for example, the effect of such treatments does not last long enough for use in hermetically capsuled small refrigerating units, which are provided with lubrication for their complete guarantee period of operation, five years.

According to the invention, it has been found that molybdenum will diffuse under the influence of elevated temperature into a ferrous metal surface which has been formed by extrusion. Apparently, a crystalline or atomic orientation occurs at such a surface, which orientation permits under the influence of elevated temperature the diffusion of molybdenum into the surface. When an article is formed by extrusion, surfaces of the article are attenuated and/or are subjected to shear by the walls of the extrusion die, the attenuation and shear occurring notably in the direction of extrusion. Accordingly, the

## 2

above referred to orientation will be in the general direction of extrusion. Furthermore, the more attenuated or subjected to shear that a given surface is by the extrusion operation, the more greatly orientated and therefore receptive to diffusion by molybdenum will the surface be.

By practicing the invention one can readily produce a molybdenum layer of for example 25 microns thickness on an extruded ferrous metal surface. This is merely exemplary. Such a layer can be readily achieved for example by the use of pure molybdenum powder, and in a small refrigerating unit piston, for example, will last for well over five years. The method of this invention is not to be confused with the known method in which the major purpose of molybdenum sulfide powder is to fill irregularities in the surface. In the present invention, there is actual diffusion of molybdenum into inter-atomic or inter-crystalline interstices. It is found that ferrous surfaces having low carbon contents are especially suitable for the method of the invention. Thus, such surfaces are iron itself or low carbon steels. However, the invention is operative with high carbon steels also.

The method of the invention is not to be confused with the alloying of tin with molybdenum in order to obtain better wearing properties and subsequently extruding the alloy. The amount of molybdenum used in this alloy is typically one half to one percent. Such alloy is harder than tin itself and is therefore less suitable for extrusion. Furthermore, it is found that the wearing properties are not significantly improved as the concentration of molybdenum is too small. Also, such an alloy does not manifest the friction reducing properties of molybdenum.

The exact temperature used for the heat treatment is not critical. In each instance, the temperature is elevated sufficiently to cause the molybdenum to diffuse into the extruded ferrous surface. Merely as an example, temperatures between about 1000° C. and 1200° C. are found to be very suitable. In order to prevent oxidation of the extruded ferrous surface or of the molybdenum during the heat treatment, it is frequently desirable to conduct the heat treatment in a reducing atmosphere such as hydrogen or in a protective atmosphere of inert gases such as nitrogen or the so-called rare or precious gases.

Generally, the best results are attained when molybdenum is used alone. However, it is not necessary to use the molybdenum alone. Accordingly, for example, the molybdenum may be used in admixture with manganese.

The molybdenum or molybdenum-containing powder may be kept in contact with the extruded ferrous surface during the heat treatment by being allowed to rest on the surface or a substance may be used to adhere the powder to the surface. The substance may for example be petroleum oil, a synthetic resin such as an epoxy resin, a natural resin, or any other material which will adhere the powder to the surface.

The method according to the invention of treating an extruded ferrous metal surface may be carried out simultaneously with other treating or fabricating operations. Thus, for example, an article having a surface to be treated by the invention may be joined with solder to another article and a subsequent heating may accordingly be used not only to aid the diffusion of molybdenum into the surface but also to complete the soldering by fusing the solder. In this instance, a soldering oven would simultaneously bring about both the diffusion of the molybdenum into the surface and the completion of the soldering of the joint.

The invention will now be further described by reference to a specific embodiment thereof in connection with the drawing. While the invention will be described as applied to a piston it will be understood that it is applicable to other elements and devices having extruded ferrous

surfaces which are to have their frictional and wear characteristics greatly improved.

A piston 1 is extruded from a sheet of low-carbon steel into a pot-like configuration having a bottom 5 and a skirt or extension wall 6. By a subsequent operation, the free end 7 of the skirt 6 is formed inward to come into good contact with a crankshaft linkage element or scotch-yoke 3 to which it is connected by solder spots 2. In a central opening 4 of the crankshaft linkage element 3 is disposed the crank pin of a crankshaft of an engine (not shown). By this construction the piston 1 is reciprocated axially in a cylinder (not shown).

Molybdenum powder, or molybdenum trioxide powder, or a mixture of molybdenum and manganese powders (for example in the ratio 60:40 respectively) is mixed with petroleum oil or an epoxy resin as an adhering medium and is applied to the outside surfaces of the piston 1 as a layer. The joined piston 1 and crankshaft linkage element 3 are then placed in a conventional soldering oven which is heated to a temperature of about 1100° C. This heating simultaneously causes the solder spots 2 to fuse and thereby complete the soldering and also causes the powder to diffuse into the outside surfaces of the piston 1.

Actually, only the outside surface of the skirt 6 requires the treatment of the invention, as only this surface is subjected to frictional operation. The method of the invention is particularly adapted for treatment of the outer surface of the skirt 6, because the skirt 6 has been particularly greatly attenuated and its outer surface subjected to shear by the extrusion by which the piston 1 was formed and, accordingly, the outer surface of the skirt 6 is particularly susceptible to diffusion by molybdenum. This will be appreciated by considering that the sheet of steel which is extruded to form the piston 1 is extruded in a direction parallel or essentially parallel to the axis of the piston 1. The sheet of steel is initially of uniform thickness and the fact that the skirt 6 is especially greatly attenuated can be appreciated by noting that the thickness of the skirt 6 is substantially less than the thickness of the bottom 5. Since the outer surface of the bottom 5 does not require the treatment it is not necessary that this part of the outer surfaces of the piston 1 be provided with the layer of powder; however, in a mass production operation it may be more convenient simply to provide the entire outer surfaces of the piston 1 with a layer of powder rather than to segregate the outer surface of the bottom 5.

A soldering oven is normally provided with an atmosphere of protecting or reducing gas and, as noted above, this is also desirable for the treatment of the invention.

The molybdenum or molybdenum-containing powder may conveniently be applied in a mass production operation by holding the article having the surface to be treated in a fluidized bed of the powder. If desired, an adhering medium may be intermixed with the powder in the fluidized bed. Alternatively, molybdenum trioxide may be

electrolytically deposited on the surface and a reducing (e.g., hydrogen) atmosphere may be provided for the heat treatment, whereby molybdenum will diffuse into the surface.

5 The invention is not to be construed as limited to the particular forms disclosed herein, since these are to be regarded as illustrative rather than restrictive.

What I claim and desire to secure by Letters Patent is:

1. A method for introducing molybdenum into a ferrous metal surface of a piston comprising forming said piston including said surface by extrusion in a direction essentially parallel to the axis of the piston with said surface extending in a direction generally parallel to said axis, whereby said surface is more highly attenuated by said extrusion than other surfaces of the piston, contacting said surface with molybdenum, and supplying heat to said surface in contact with the molybdenum to cause diffusion of the molybdenum into said surface.

2. A method according to claim 1, wherein the heating is carried out in a protective gas atmosphere.

3. A method according to claim 1, wherein the protective gas atmosphere is a reducing atmosphere.

4. A method according to claim 1, wherein said surface is also contacted with manganese and the heat is applied while said surface is in contact both with the manganese and the molybdenum.

5. A method according to claim 1, wherein the molybdenum is held in contact with said surface with an adhesive.

6. A method according to claim 1, wherein said piston is joined with solder to an article and heat is supplied to the solder simultaneously with the heating of said surface, whereby in a single operation the molybdenum is caused to diffuse into said surface and the solder is fused to complete the joining with solder.

7. A method according to claim 1, wherein the piston is joined with solder to a crankshaft linkage element, before said surface is supplied with heat while in contact with the molybdenum.

40

#### References Cited

##### UNITED STATES PATENTS

|           |         |                      |            |
|-----------|---------|----------------------|------------|
| 1,717,750 | 6/1929  | Wills -----          | 29—156.5   |
| 2,201,405 | 5/1940  | McCarroll -----      | 92—223     |
| 2,410,405 | 11/1946 | Cornelius -----      | 92—223 X   |
| 2,817,562 | 12/1957 | Fleming et al. ----- | 29—156.5   |
| 2,833,264 | 5/1958  | Dailey et al. -----  | 29—156.5   |
| 2,833,668 | 5/1958  | Dailey et al. -----  | 29—156.5   |
| 2,984,895 | 5/1961  | Griffin et al. ----- | 29—156.5 X |
| 3,041,194 | 6/1962  | Rosen et al. -----   | 29—156.5   |

##### FOREIGN PATENTS

|           |        |          |
|-----------|--------|----------|
| 1,037,220 | 8/1958 | Germany. |
|-----------|--------|----------|

55 JOHN F. CAMPBELL, Primary Examiner.

P. M. COHEN, Assistant Examiner.